

3,547,820

**LUBRICATING OIL COMPOSITIONS**

Fred E. Woodward, Plainfield, N.J., and William Katzenstein, Broomall, Pa., assignors to GAF Corporation, New York, N.Y., a corporation of Delaware  
No. Drawing. Continuation of application Ser. No. 583,097, Sept. 29, 1966, which is a continuation-in-part of application Ser. No. 203,007, June 18, 1962, which in turn is a continuation-in-part of application Ser. No. 154,834, Nov. 24, 1961. This application Dec. 20, 1968, Ser. No. 786,848

Int. Cl. C10m 1/46

U.S. Cl. 252—32.5

8 Claims

**ABSTRACT OF THE DISCLOSURE**

A mineral lubricating oil composition containing about 0.5% to about 25% by weight of a material selected from a phosphate ester and a salt of a phosphate ester of phosphoric acid and an oxyalkylene ether of an organic hydroxy compound. The organic hydroxy compound is selected from alkyl phenols and aliphatic straight chain alcohols, the phosphate ester being selected from monoesters, diesters and mixtures thereof, the oxyalkylene group of the oxyalkylene ether comprising a maximum of about 50% by weight thereof.

This application is a streamlined continuation of application Ser. No. 583,097, filed Sept. 29, 1966, now abandoned, which in turn is a continuation-in-part of application Ser. No. 203,007 filed June 18, 1962, now abandoned, which in turn is a continuation-in-part of application Ser. No. 154,834 filed Nov. 24, 1961, now abandoned.

This invention relates to improved lubricating oil compositions, and more particularly to detergent mineral oil lubricating compositions for use in internal combustion engines, which compositions have outstanding antiwear properties.

It is well known that lubricating oils commonly used in internal combustion engines and which are derived from the refining of mineral oils undergo considerable oxidation and degradation during use in an engine. This oxidation of the oil produces sludge deposits which may cause the various parts of the engine to operate inefficiently. In order to overcome such conditions, detergent lubricating oils have been developed which have the ability to suspend the aforementioned sludge materials and keep them from interfering with the normal and efficient operation of the engine. Other additives have been developed for use in such oil compositions to improve the lubricating characteristics thereof and thereby lessen the wear of the engine parts. The present invention is concerned with the discovery of a class of additives which exhibits not only outstanding detergent characteristics but also excellent antiwear properties.

It is therefore an object of the present invention to provide a lubricating oil composition which has outstanding detergent characteristics.

It is another object of the present invention to provide a lubricating oil composition which has excellent and improved antiwear properties.

It is still another object of the present invention to provide a mineral oil lubricating oil composition which is characterized by outstanding detergent and antiwear properties.

It is still another object of the present invention to provide a mineral oil lubricating composition particularly adaptable for use in internal combustion engines and which has improved detergent and lubricating properties.

It is still another object of the present invention to provide a mineral oil lubricating composition particularly

adapted for use in internal combustion engines which is characterized by outstanding detergent and antiwear properties.

Other objects will appear as the description proceeds.

The compositions of the present invention comprise the usual mineral lubricating oils on the one hand which may also contain the conventional modifiers and additives in minor amounts such as synthetic lubricating oils, viscosity index improvers, corrosion inhibitors, pour depressants, dyes and the like, and a phosphate ester of a nonionic surface active agent more sufficiently described below.

The phosphate esters of nonionic surface active agents which are herein contemplated are mono- and diphosphate esters and mixtures thereof. The nonionic precursors for the esters are selected from the group consisting of polyoxyalkylene ethers of alkyl phenols and aliphatic alcohols of at least 15 carbon atoms, said oxyalkylene groups containing from 2 to 3 carbon atoms each. The amount of oxyalkylene groups may vary from about 10% (i.e., derived from the interaction of 1 mole alkylene oxide) up to 50% by weight alkylene oxide. The alkylene oxides or precursors thereof which may be employed to yield the corresponding oxyalkylene groups in the nonionic surface active agent are those which contain from 2 to 3 carbon atoms such as ethylene oxide, propylene oxide, and the like. In addition, it is clear and obvious that mixtures of such oxyalkylating reagents may be used whereby there results in the nonionic surfactant, variations in the oxyalkylene groups.

The nonionic oxyalkylated products which are herein contemplated as precursors for the phosphate esters are well known in the art and are derived from alkyl phenols and aliphatic alcohols of at least 15 carbon atoms and the alkylene oxide as, for example, disclosed in U.S. Pats. 2,213,477 and 1,970,578. The following illustrate some typical suitable phenols and alcohols which may be used to form the corresponding nonionic surface active agents which are precursors for the instantly contemplated phosphate esters:

40 nonyl phenol (nonyl derived from propylene trimer)  
dodecyl phenol (derived from propylene tetramer)  
hexadecyl phenol  
octadecyl phenol,

45 and the like phenols containing a plurality of different alkyl groups, for example:

butyl amyl phenol  
butyl hexyl phenol  
50 amyl hexyl phenol  
amyl heptyl phenol  
ethyl heptyl phenol

as well as phenols containing a plurality of similar alkyls such as, in addition to those above:

di-n-hexyl phenol  
diisohexyl phenol  
di-n-heptyl phenol  
60 di-n-octyl phenol  
diiso-octyl phenol  
dinonyl phenol  
didodecyl phenol  
ditetradecyl phenol  
65 diocta decyl phenol  
tri-n-octyl phenol  
tri-n-butyl phenol, and the like, and

70 alcohols prepared from olefins from C<sub>12</sub> to C<sub>50</sub> by the "oxa" process.

The above compounds are then reacted with the alkylene oxide as described above to yield the nonionic sur-

face active agents which are then used to prepare phosphate esters employed in the compositions of the present invention.

The phosphate esters may be prepared by the reaction of 1 mol of  $P_2O_5$  with 2 to 4.5 mols of the nonionic surfactant as described and claimed in U.S. Patent 3,004,056 by Nunn and Hesse and U.S. Patent 3,004,057 by Nunn. As described in the said Nunn and Hesse patent, the reaction between the  $P_2O_5$  and the nonionic polyoxyalkylene ether is conducted under substantially anhydrous conditions and at a temperature below about 110° C. In its preferred form, the reaction is carried out by adding the  $P_2O_5$  gradually, with vigorous agitation to the nonionic surface active agent in liquid form. The reaction is exothermic and cooling is in some cases necessary to keep the temperature below 110° C., since discolored and darkened products tend to be produced above this temperature. The reaction proceeds continuously during the addition of the  $P_2O_5$  and is preferably followed by maintenance of the reaction mixture at ambient temperatures up to 110° C. for an additional period of time after completion of such addition to allow for complete solution of the  $P_2O_5$  and reaction with the nonionic surface active agent.

The following examples illustrate the preparation of such phosphate esters.

#### Example A

2.7 mols of a nonionic surface active compound derives from dinonyl phenol condensed with 4 mols of ethylene oxide is reacted with 1 mol of  $P_2O_5$  in the manner described in the examples of U.S. Pat. 3,004,056. The product consists of about equal amounts of mono- and diester with about 10-15% unreacted nonionic.

#### Example B

The procedure of Example A is repeated except that the nonionic is a dodecyl phenol plus 2 mols of ethylene oxide condensate.

#### Example C

The procedure of Example A is again repeated employing as the nonionic surface active agent a dinonyl phenol plus 5 mols ethylene oxide (40% ethylene oxide content).

#### Example D

The procedure of Example A is once again repeated employing as the surfactant a dinonyl phenol plus 7 mols ethylene oxide (47% ethylene oxide content).

#### Example E

The procedure of Example A is still once again repeated employing as the nonionic surface active agent dinonyl phenol reacted with 1.5 mols of ethylene oxide to yield a nonionic product containing about 20% ethylene oxide.

#### Example F

The above procedures are again repeated using as the nonionic precursor the condensation product of dodecyl phenol with 1.8 mol of ethylene oxide.

The chemical constitution of the products produced in the above described examples will usually be about 20 to 50% of the secondary phosphate ester of the nonionic agent, 30 to 80% of the primary phosphate ester, and 0 to 40% of unreacted nonionic agent.

By carrying out the above reaction in the presence of a small amount of a phosphorus-containing compound selected from the group consisting of hypophosphorous acid, salts of hypophosphorous acid, phosphorous acid, and salts and esters of phosphorous acid, preferably sodium hypophosphite or hypophosphorous acid, as described in said Nunn '057 patent, lighter colored or substantially colorless reaction products are obtained.

While the presence of unreacted nonionic is not detrimental to the attainment of the objects of the present invention, the amount of nonionic can be reduced, if desired, to a minimum of less than about 10% by incorporating in the reaction mixture a small amount of mineral acid as phosphoric acid, hydrochloric acid or sulfuric acid. Since phosphorous pentoxide yields phosphoric acid in the presence of water, the latter can advantageously and preferably be used to form the acid "in situ." With the use of the mineral acid the amount of phosphorous pentoxide can also be increased to as much as 3 mols per mol of nonionic reactant, thereby favoring the formation of the monoester in major amounts, i.e., substantially no diester.

15 Monoesters and diesters can also be prepared from the corresponding triesters by reacting the triester with phosphoric acid. By varying the ratio of nonionic to acid, one can prepare either mono- or diester to the substantial exclusion of the other. A high ratio of triester to acid (2:1) produces diester whereas a low ratio (0.5:1) produces monoester.

#### Example G

25 Equimolar amounts of the nonionic surface active compound of Example A and phosphorous pentoxide are heated at 90° C., while adding in the presence of about 0.4% water the  $P_2O_5$  over a period of one hour. Then the reaction mixture is heated for 4 hours at 125° C. The final product is a monoester.

#### Example H

30 Example G is repeated employing one mol of a dodecyl phenol plus 2 mols ethylene oxide condensate and 2 mols of  $P_2O_5$ . The final product is a monoester.

#### Example I

35 Example G is again repeated using the following non-  
ionics:

- (A) octadecanol + 2 mols ethylene oxide
- (B) hexadecanol + 4 mols ethylene oxide
- (C) 1-eicosanol + 6 mols ethylene oxide
- (D) 1-dotriacontanol + 7 mols ethylene oxide
- (E) dodecyl phenol + 5 mols ethylene oxide
- (F) hexadecyl phenol + 3 mols ethylene oxide
- (G) tri-n-octyl phenol + 4 mols ethylene oxide
- (H) tri-n-octyl phenol + 5 mols propylene oxide
- (I) dodecyl phenol + 3 mols propylene oxide
- (J) dinonyl phenol + 1.5 mols propylene oxide
- (K) diisohexyl phenol + 2 mols propylene oxide
- (L) tri-n-butyl phenol + 2 mols propylene oxide
- (M) tri-n-butyl phenol + 3 mols propylene oxide
- (N) tri-n-butyl phenol + 4 mols propylene oxide
- (O) tri-n-butyl phenol + 3 mols ethylene oxide
- (P) hexadecanol + 3 mols propylene oxide
- (Q) octadecanol + 4 mols propylene oxide
- (R) butyl hexyl phenol + 4 mols ethylene oxide
- (S) ethyl heptyl phenol + 5 mols ethylene oxide
- (T) ethyl heptyl phenol + 3 mols propylene oxide
- (U) cetyl alcohol + 2 mols ethylene oxide
- (V) 1-octacosanol + 4 mols ethylene oxide
- (W) 1-nonacosanol + 7 mols ethylene oxide
- (X) 1-triacontanol + 6 mols ethylene oxide
- (Y) 1-tetratricacontanol + 5 mols ethylene oxide
- (Z) 1-tetratricacontanol + 2 mols propylene oxide

#### Example J

70 A phosphate triester of the nonionic compound of Example A is prepared by reacting 3 mols of said nonionic with 1 mol of phosphorous oxychloride in the presence of 1 mol of pyridine and 100 ml. of benzene. The  $POCl_3$  is added dropwise to the other components at a temperature of about 0° C. and the temperature is held below 10° C. After all of the  $POCl_3$  has been added, the mixture is refluxed for 3 hours and then the solvent is removed 75 under vacuum distillation. The triester results.

The triester is converted to a monoester by adding 1 mol of phosphoric acid to 0.5 mol of the triester at about room temperature. The monoester results.

Example K

Example J is repeated except that 2 mols of triester are used in lieu of 0.5 mol. The diester results.

The mono- and di-phosphated products may be represented by the following formulae:



wherein R' represents H, or methyl; X may be hydrogen, alkali metal, alkaline earth metal, e.g., calcium, magnesium, barium, etc., ammonium, amine or substituted ammonium and amine, and n equals the number of mols of alkylene oxide necessary to yield a final product containing up to 50% by weight of the said alkylene oxide as discussed above; R is the alcohol or phenol hydrophobe nucleus. It is preferred that X be other than hydrogen.

The detergents which have been used heretofore in lubricating oils are in the main metal sulfonates which, however, have only marginal performance in internal combustion engines. The phosphate esters herein contemplated have superior detergent properties as evidenced by the following data. In the examples which are given below, parts are by weight unless otherwise indicated. These examples are by way of illustration only and are not to be deemed limitative of the present invention.

Example 1

The oil used in the detergency test is a standard S.A.E. 20 oil which has been used 2000 miles and which contains no additives. The sediment in the oil is given in milliliters and the ratings are:

- 1-0.05 ml.=excellent  
2-0.3 ml.=average  
3-3 ml.=poor

The physical appearance of the supernatant oil is reported as follows:

- (1) 1—opaque—good  
(2) 2—hazy—average  
(3) 3—clear—poor

A good dispersant should have a rating of (1), i.e., .05 ml. sediment, while an average oil falls into the range of 2 to 0.3 ml.

TABLE I.—DETERGENCY TEST

|                                                                                                                       | Percent<br>wt.<br>additive | Oil<br>appear-<br>ance | Sedi-<br>ment | 65 |
|-----------------------------------------------------------------------------------------------------------------------|----------------------------|------------------------|---------------|----|
| (1) Oil (no additive)                                                                                                 |                            | 8                      | 3             |    |
| (2) (1) plus basic barium wax benzene<br>high boiler sulfonate                                                        | 3.3                        | 2                      | 2             |    |
| (3) (1) plus basic calcium dinonyl naph-<br>thalene sulfonate                                                         | 3.3                        | 2                      | 2             | 70 |
| (4) (1) plus barium salt of complex phos-<br>phate ester of dinonyl phenol plus 4<br>mols ethylene oxide of Example A | 3.3                        | 1                      | 1             |    |
| (5) (1) plus barium salt of complex phos-<br>phate ester of dodecyl phenol plus 2<br>mols ethylene oxide of Example B | 3.3                        | 1                      | 1             |    |

Example 2

The outstanding anti-wear properties of the compositions of the present invention are demonstrated on the Shell Four Ball Machine (Brown—G.E. modification using 4 steel balls). The oil used is a 150 S.A.E. at 100° F. solvent refined Mid Continent oil.

10 TABLE II.—SHELL FOUR BALL WEAR TEST  
[1 hour, 600 r.p.m. at 200° F.]

| 15                                                                                                                              | Composition | Sear size,<br>mm. |        | Coefficient of<br>friction |        |
|---------------------------------------------------------------------------------------------------------------------------------|-------------|-------------------|--------|----------------------------|--------|
|                                                                                                                                 |             | 20 kg.            | 50 kg. | 20 kg.                     | 59 kg. |
| (A) Unmodified oil                                                                                                              |             | 0.7               | 0.9    | 0.125                      | 0.09   |
| (B) (A) plus 3.3% basic barium wax<br>benzene high boiler sulfonate                                                             |             | 0.6               | 0.75   | 0.10                       | 0.005  |
| (C) (A) plus 3.3% basic calcium dinonyl<br>naphthalene sulfonate                                                                |             | 0.65              | 0.80   | 0.12                       | 0.09   |
| (D) (A) plus 3.3% barium salt of com-<br>plex phosphate ester of dinonyl phenol<br>plus 4 mols ethylene oxide of Ex-<br>ample A |             | 0.25              | 0.35   | 0.072                      | 0.052  |
| (E) (A) plus 3.3% barium salt of com-<br>plex phosphate ester of dodecyl phenol<br>plus 2 mols ethylene oxide of Example<br>B   |             | 0.20              | 0.45   | 0.032                      | 0.096  |

25 Example 3

30 The barium salt of the phosphate ester is prepared in general by heating the compounds of Formulae I and II preferably in the form of the free acid with barium hydroxide in mineral oil. Thus, 100 grams of a complex phosphate ester of dinonyl phenol containing 40% ethylene oxide (as the free acid form) is heated with agitation at 85° C. with 100 grams of 150 second solvent and refined neutral mineral oil. Then 34 grams of



35 is slowly added over a 10 minute period. Agitation is continued for 1 hour at 85° C. and then the mixture is cooled. The final product is clear and has a pH of 10.2 as a 5% solution in isopropanol.

40 Example 4

45 Examples 1 and 2 are repeated employing the potassium salt of the phosphate esters. Such salts are prepared by neutralizing the free acid in situ with 50% KOH to a pH of about 6.0. Similar outstanding results are obtained.

Example 5

50 In this example, Examples 1 and 2 are repeated using dinonyl phenol-ethylene oxide condensates as the non-ionic precursors for the phosphate esters containing varying ethylene oxide content as indicated.

|   | Mols Et <sub>2</sub> O | Percent<br>Et <sub>2</sub> O<br>on wt. of<br>non-ionic<br>produced |
|---|------------------------|--------------------------------------------------------------------|
| A | 1                      | 11                                                                 |
| B | 2                      | 20                                                                 |
| C | 4                      | 34                                                                 |
| D | 6                      | 43                                                                 |

60 Excellent results are obtained with the barium salts of the complexes.

65 In the following examples Example 2 is repeated using the indicated non-ionics. The salts thereof are also indicated.

| Non-ionic                                      | Mols alkylene oxide | Alkylene percent oxide | Salt                                                                                                         |
|------------------------------------------------|---------------------|------------------------|--------------------------------------------------------------------------------------------------------------|
| Example:                                       |                     |                        |                                                                                                              |
| 6..... Nonyl phenolethylene oxide.....         | 1                   | 16.7                   | {(a) Ba.<br>(b) Ca.<br>(c) Cd.<br>(d) Ethylamine.                                                            |
| 7..... do.....                                 | 5                   | 50                     | {(a) Ba.<br>(b) K.<br>(c) NH.<br>(d) Monoethanolamine.                                                       |
| 8..... Dodecyl phenolethylene oxide.....       | 1.8                 | 23.2                   | {(a) Ba.<br>(b) Zn.<br>(c) Mg.<br>(d) Ethylene diamine.<br>(e) Monoethanolamine.<br>(f) Diethylene triamine. |
| 9..... Nonyl phenolpropylene oxide.....        | 3.0                 | 44                     | {(a) Ba.<br>(b) Ca.                                                                                          |
| 10..... Hexadecyl phenolethylene oxide.....    | 3.0                 | 30                     | {(a) Ca.<br>(b) Zn.<br>(c) K.<br>(d) Ethylenediamine.                                                        |
| 11..... tri-n-Butyl phenolethylene oxide.....  | 3.0                 | 33                     | {(a) Ba.<br>(b) Zn.                                                                                          |
| 12..... tri-n-Butyl phenolpropylene oxide..... | 2.0                 | 31                     | {(a) Ba.<br>(b) Mg.<br>(c) NH <sub>4</sub> .                                                                 |
| 13..... Hexadecanolethylene oxide.....         | 4.0                 | 42                     | {(a) Zn.<br>(b) Ba.<br>(c) Ca.                                                                               |
| 14..... Octadecanolpropylene oxide.....        | 4.0                 | 46                     | {(a) K.<br>(b) Mg.<br>(c) Ca.<br>(d) Zn.                                                                     |

The above non-ionics are phosphated before salt formation using the techniques of Example A.

about 45% diester, about 35% monoester and about 20% unreacted non-ionic.

#### Example 15

A monoester as in Example G is used as in Example 2 as the barium salt. Comparable results are achieved.

Example 17 is repeated using the following ratios of non-ionic to P<sub>2</sub>O<sub>5</sub>:

40

|          | Ratio | Percent monoester | Percent diester |
|----------|-------|-------------------|-----------------|
| Example: |       |                   |                 |
| 18.....  | 2.0   | 75                | 20              |
| 19.....  | 2.5   | 60                | 30              |
| 20.....  | 3.0   | 40                | 40              |
| 21.....  | 3.5   | 40                | 45              |
| 22.....  | 4.2   | 32                | 48              |
| 23.....  | 4.5   | 30                | 50              |

#### Example 24

50 The "Four-Ball" wear test of Example 2 is repeated using the indicated compounds and conditions:

Conditions: 1 hour—100 r.p.m. at 250° F.

Base oil: solvent refined, 100 SUS, neutral

| Compound                                       | Conc. percent | Load              |                     |        |        |         |        |
|------------------------------------------------|---------------|-------------------|---------------------|--------|--------|---------|--------|
|                                                |               | 40 kg.            |                     | 60 kg. |        | 100 kg. |        |
|                                                |               | S.D. <sup>1</sup> | C.O.F. <sup>2</sup> | S.D.   | C.O.F. | S.D.    | C.O.F. |
| (a) Base oil.....                              |               | 0.50              | 0.14                | 0.60   | 0.13   | 0.75    | 0.14   |
| (b) Ex. A but 1.8 mols E.O. <sup>3</sup> ..... | 1.0           | 0.35              | 0.100               | 0.40   | 0.085  | 0.55    | 0.094  |
| (c) Same as (b) but barium salt.....           | 1.0           | 0.50              | 0.105               | 0.60   | 0.082  | 0.65    | 0.086  |
| (d) Ex. D.....                                 | 1.0           | 0.45              | 0.123               | 0.50   | 0.098  | 0.50    | 0.110  |
| (e) Ba salt of Ex. D.....                      | 1.0           | 0.60              | 0.082               | 0.60   | 0.090  | 0.65    | 0.089  |
| (f) Basic Ba salt of Ex. D.....                | 1.0           | 0.50              | 0.117               | 0.60   | 0.078  | 0.70    | 0.089  |
| (g) Chlorinated paraffin wax (40% Cl).....     | 2.0           | 0.50              | 0.053               | 0.62   | 0.062  | 0.64    | 0.080  |
| (h) Trilaurylthiophosphate.....                | 2.0           | 0.50              | 0.097               | 0.80   | 0.094  | (4)     | —      |
| (i) Tricresyl phosphate.....                   | 2.0           | 0.55              | 0.088               | 0.60   | 0.098  | (4)     | —      |

<sup>1</sup> Scar diameter (mm.).

<sup>2</sup> Coefficient of friction.

<sup>3</sup> Ethylene oxide.

<sup>4</sup> Welded.

**9**  
Example 25

The product of Example 24(c) is tested in the following composition in a MS-Sequence I, II, and III (Oldsmobile):

Composition  
Base oil: SAE 10W-30  
Solvent: Refined Mid-Continent

|                                                       | Percent by volume | 5  |
|-------------------------------------------------------|-------------------|----|
| Product of Ex. 24(c)                                  | 1.3               | 10 |
| Zinc dihexyl dithiophosphate (8% P; 16.1% S; 818% Zn) | 0.6               |    |
| V.I. improver (polyalkylmethacrylate)                 | 4.50              |    |

The performance levels (based on a 0 to 10 scale with 10 being perfect) are:

|                        |      |
|------------------------|------|
| Varnish deposit:       |      |
| Piston skirts, Aug.    | 9.5  |
| Rocker arm cover plate | 9.5  |
| Top cover              | 9.5  |
| Cylinder walls (BRT)   | 9.5  |
| Crankcase oil pan      | 9.5  |
| Varnish average        | 9.5  |
| Sludge deposit:        |      |
| Rocker arm plate       | 10.0 |
| Top cover              | 10.0 |
| Oil screen             | 10.0 |
| Crankcase oil pan      | 9.0  |
| Average sludge         | 9.8  |
| Ring evaluation:       |      |
| Ring sticking          | None |
| Oil ring plugging      | None |
| Scuffing:              |      |
| Valve lifter           | None |
| Cam lobes              | None |

Example 26

The product of (a) Example D (phosphated dinonyl phenol+7 mols ethylene oxide condensate) and (b) a tallow alcohol ( $C_{18}$ -50% unsaturated)+2 mols ethylene oxide condensate phosphated similarly as in Example D are tested on a "Falex" Wear Test apparatus in a 150 SUS paraffinic base oil.

Conditions: Load-1000 lbs.  
Time: 2 minutes each at 250, 500, and 750 lbs. and 15 minutes at 1000 lbs.  
Speed: 290 r.p.m.  
Temperature: 175° F.

**10**

| Product base oil: | Total no. of teeth <sup>1</sup> failure during initial trial in period at 250 lbs. Pin appearance |
|-------------------|---------------------------------------------------------------------------------------------------|
| 0.5% (a)          | 3 Very smooth, shiny.                                                                             |
| 1.0% (a)          | 3 Do.                                                                                             |
| 2.5% (a)          | 8 Do.                                                                                             |
| 0.5% (b)          | 9 Smooth, shiny.                                                                                  |
| 1.0% (b)          | 9 Slight ridging, shiny.                                                                          |
| Commercial Oil A  | 320 Severe chewing, black.                                                                        |

<sup>1</sup> Each tooth is equivalent to 0.000056 inch wear.

Example 27

B-10-A oxidation corrosion test is run on the indicated products using the following setup.

Into a 100 ml. test tube, there are placed, sanded and solvent cleaned:

- (1) coil of mild steel SAF-1010 wire  $2\frac{3}{4}$ " long and  $\frac{1}{2}$ " in diameter;
  - (2) 4" long piece of copper wire 0.1 mm. in diameter bent double and placed half inside and half outside steel coil; and
  - (3) 3" long piece of aluminum wire 0.2 mm. in diameter bent double and placed inside steel coil
- 25 Liquid to be tested is added to cover all metal and then a glass tube 0.4 mm. in diameter and  $9\frac{1}{2}$ " long is placed into test tube and a glass cover with hole in center to accommodate glass tube is placed to rest on top of test tube with glass tube centered in test tube through hole in cover. This setup is placed in an oil bath at 250° F. with the oil lever being above the level of the test liquid. An air supply running through a silica drying filter and control manifold is fed to the glass tube. Air flow is 10 liters/hour and test is run for 72 hours.
- 30 In the table the numerical values for sludge and discoloration have the following significance:
- Sludge rating:
- (1) No sludge
  - (2) Trace sludge
  - (3) Medium sludge
  - (4) Severe sludge
- 45 Discoloration scale:
- (1) No staining
  - (2) Slight staining
  - (3) Medium staining
  - (4) Severe staining
- 50

TABLE

| Composition                                                                                                             | Sludge rating | Discoloration |    |    |
|-------------------------------------------------------------------------------------------------------------------------|---------------|---------------|----|----|
|                                                                                                                         |               | Cu            | Al | Fe |
| Base oil plus 3% Ba salt of tridecyl alcohol plus 3 E.O. phosphated as in Ex. A plus 0.75% zinc dihexyl dithiophosphate |               | 4             | 4  | 3  |
| Base oil plus 3% Ba salt dodecyl phenol plus 1.5 E.O. phosphated as in Ex. A plus 0.75% zinc dihexyl dithiophosphate    |               | 1             | 2  | 1  |
| Base oil plus 7% t-butylamine salt of dinonyl phenol plus 2 E.O. phosphated as in Ex. A                                 |               | 2             | 1  | 1  |
| Base oil plus 3% sodium salt of tallow alcohol plus 2 E.O. phosphated as in Ex. A                                       |               | 2             | 1  | 1  |
| Base oil plus 3% barium salt of phenol plus 4 E.O. phosphated as in Ex. A                                               |               | 4             | 4  | 4  |
| Base oil plus 3% barium salt of phenol plus 4 E.O. phosphated as in Ex. A plus 0.75% zinc dihexyl dithiophosphate       |               | 4             | 4  | 4  |

## 11

## Example 28

The barium salt prepared in Example 3 is compounded (A) with a typical engine oil as follows:

To the solvent refined base there is added 3.3% barium salt of Example 3, 0.75% zinc dialkyl dithiophosphate and 6.6% Acryloid 966 (copolymer of lauryl methacrylate (90%) and vinyl pyrrolidone 10%). A similar composition (B) is prepared except that the detergent used is 3.3% of the barium salt of wax benzene high boiler sulfonate. In a Shell Four Ball Test as previously described the results are:

| Composition: | mm. Scar size |        |
|--------------|---------------|--------|
|              | 20 kg.        | 50 kg. |
| A            | 0.20          | 0.40   |
| B            | 0.35          | 0.55   |

## Example 29

Example 24 is repeated using 3% by weight based on the weight of the base oil of the following amine salts:

| Non-Ionic                           | Mols<br>alkylene<br>oxide | Alkylene<br>oxide,<br>percent | Phosphation<br>procedure | Amine               |
|-------------------------------------|---------------------------|-------------------------------|--------------------------|---------------------|
| Nonyl phenol ethylene oxide         | 5                         | 50                            | Example A                | Monoethanolamine.   |
| Do                                  | 1                         | 16.7                          | do                       | Ethylamine.         |
| Dodecyl phenoxyethylene             | 1.8                       | 23.2                          | do                       | Ethylenediamine.    |
| Do                                  | 1.8                       | 23.2                          | do                       | Monoethanolamine.   |
| Do                                  | 1.8                       | 23.2                          | do                       | Diethylenetriamine. |
| Hexadecyl phenoxyethylene<br>oxide. | 3.0                       | 30                            | do                       | Ethylenediamine.    |
| Hexadecanoleethylene oxide          | 4.0                       | 42                            | do                       | Triethylenediamine. |

Excellent anti-wear properties are evidenced by the low scar diameters produced.

The amine salts are prepared preferably in the mineral oil base using, in general, sufficient amine to neutralize the acid group of the phosphate non-ionic compound. All of the salts contemplated herein may also be produced in any suitable non-reactive solvent medium or even in the absence of a solvent or diluent, e.g., where the amine is a liquid.

## Example 30

In a Falex Wear Test carried out as in Example 26, the products of Example 29, at concentrations of 0.5% and 1% by weight based on the weight of the oil all showed a total of teeth failed to be less than 10 during the 250 lb. load.

As described above, the usual additives may be employed with the improved detergent oils herein disclosed. These include viscosity index improvers such as polyisobutylene, pour point depressants, blooming agents, peptizing agents, other detergents, anti-oxidants and the like.

The concentration of phosphate ester in the mineral lubricating oils may range from about 0.5% to about 25% by weight based on the weight of the oil.

Other variations in and modifications of the described processes which will be obvious to those skilled in the

## 12

art can be made in this invention without departing from the scope or spirit thereof.

We claim:

1. A mineral lubricating oil composition containing from about 0.5% to about 25% by weight based on the weight of the oil of a phosphate ester, in the form of its free acid or alkali metal, alkaline earth metal or ammonium salt, of an oxyalkylene ether of an organic hydroxy compound containing at least 15 carbon atoms and selected from the group consisting of alkylphenols and aliphatic straight chain alcohols, said phosphate ester being selected from the group consisting of monoesters, diesters and mixtures thereof, said oxyalkylene ether containing at least one oxyalkylene group of 2 to 3 carbon atoms and a maximum of 50% by weight of oxyalkylene groups, each of from 2 to 3 carbon atoms, based on the weight of said oxyalkylene ether.
2. A composition as defined in claim 1 wherein said organic hydroxy compound is an alkylphenol.
3. A composition as defined in claim 1 wherein said organic hydroxy compound is an aliphatic straight chain alcohol.

4. A composition as defined in claim 1 wherein said oxyalkylene groups are oxyethylene groups.

5. A composition as defined in claim 1 wherein said phosphate ester is employed in the form of its free acid.

6. A composition as defined in claim 1 wherein said phosphate ester is employed in the form of its alkali metal salt.

7. A composition as defined in claim 1 wherein said phosphate ester is employed in the form of its alkaline earth metal salt.

8. A composition as defined in claim 1 wherein said phosphate ester is employed in the form of its ammonium salt.

## References Cited

## UNITED STATES PATENTS

- 2,848,414 8/1958 Chenicek \_\_\_\_\_ 252—32.5  
2,961,408 11/1960 Havely et al. \_\_\_\_\_ 252—32.5  
3,033,889 5/1962 Chiddix et al. \_\_\_\_\_ 252—49.8

55 PATRICK P. GARVIN, Primary Examiner

I. VAUGHN, Assistant Examiner

U.S. Cl. X.R.

60 252—49.8